

## UNITED STATES PATENT OFFICE

2,066,216

## LUBRICATING COMPOSITION

Floyd L. Miller, Roselle Park, N. J., and Arnold J. Morway, New York, N. Y., assignors to Standard Oil Development Company, a corporation of Delaware

No Drawing. Application June 29, 1933,  
Serial No. 678,188

4 Claims. (Cl. 87—9)

This invention relates to improved lubricating compositions, particularly compositions of the general nature of greases or of compounded oils which are suitable for lubricating gears and surfaces especially where high pressures are maintained.

Greases are manufactured by incorporating soaps such as potassium, sodium, calcium, or similar soaps, into a lubricating oil at elevated temperatures. On cooling this mixture, a structure is obtained in which lubricating oil is held in rigid form by virtue of the interlacing structure of the soaps. On prolonged storage, especially where temperatures above 80° F. are maintained, this composition tends to break in that it sweats or allows the oil to run out from the structure. Similarly, compounded oils manufactured by blending a mineral lubricating oil and certain metallic soaps such as, for example, lead oleate, when first compounded are usually clear and homogeneous but upon standing often have a tendency to separate and settle out into two layers.

An object of this invention is to stabilize such greases and compounded oils.

Another object of this invention is to stabilize greases or compounded oils that are of known lubricating value without materially changing their lubricating qualities.

These and other objects of the invention will be seen in the following description of our invention.

It has been discovered that some metallic soaps possess the unusual property of forming colloids of the type known as "emulsoidal" when added to a hydrocarbon oil. These metallic soaps in many cases appear at first to be perfectly oil-soluble but immediately begin to form colloids homogeneously dispersed throughout the entire mass of the oil. In other cases, it may be necessary to use heat to effect solution, after which the mixture is cooled. Such metallic soap colloids are stable, in that they do not settle out from the oil on standing even at elevated temperatures and their behavior appears to be of a similar nature to that of a gelatin dissolved in water.

These metallic soaps, which form emulsoidal colloids when added to a lubricating oil, are added to a grease containing an alkali or an alkali earth soap which tends to separate or sweat and the resulting mixture is stabilized so that sweating does not take place on standing over a prolonged period of time, or it is minimized especially when the grease is subjected to temperatures above 80° F., as sweating of a grease most often takes place at these temperatures. These metallic soaps also stabilize compounded oils, i. e., oils that contain more or less soluble metallic soaps, such as lead oleate, which tend to partially separate on standing.

The quantity of metallic soaps that is usually added is about 1%, though up to 2½% has been added without materially changing the physical characteristics of the lubricating compositions. The metallic soaps which have been discovered to have the desired property of forming emulsoidal colloids when dissolved in a mineral lubricating oil are cobalt and cadmium soaps of unsaturated acids such as oleic and linoleic acids and certain types of naphthenic acids. Of especial value are the acids recovered from the product obtained by cracking crudes containing naphthenic acids. Although their true structure is uncertain, they will be included in the term "naphthenic acids". Especially suitable are the synthetic acids prepared by the oxidation of paraffin wax.

The invention will be more readily understood from the following examples:

10 pounds of a fatty oil such as prime tallow, 20 or mixed fats, and 48.5 pounds of mineral lubricating oil having a Saybolt viscosity of about 100 seconds at 100° F. are mixed and the mixture is heated to about 280° F. The heating is continued and a mixture of 1.25 pounds of water and 1.40 pounds of hydrated lime (23.5% water of hydration) is slowly added with constant stirring until all of the fatty oil is saponified and part of the water driven off. Then 1 pound of manganese linoleate or cadmium stearate soap is incorporated. The resulting product has the following composition:

|                                         | Per cent |
|-----------------------------------------|----------|
| Calcium soap                            | 18.02    |
| Water                                   | 0.50 35  |
| Mineral lubricating oil                 | 80.48    |
| Manganese linoleate or cadmium stearate | 1.00     |

An alternate method of preparing a grease is as follows:

3 pounds of stearic acid, 8 pounds of oleic acid, and 86.5 pounds of mineral lubricating oil having a Saybolt viscosity of 300 to 400 seconds at 100° F. are mixed. The mixture is slowly heated to about 250° F. and 2 pounds of a water mixture of hydrated lime is slowly added with constant stirring until the saponification is completed and nearly all of the water driven off. Then 2 pounds of either cadmium oleate or cobalt naphthenate is incorporated. The resulting product has the following composition:

|                         | Per cent |
|-------------------------|----------|
| Calcium oleate          | 8.0      |
| Calcium stearate        | 3.0      |
| Mineral lubricating oil | 86.5 55  |
| Cadmium or cobalt soap  | 2.0      |
| Water                   | 0.5      |

The methods of incorporating the metallic soaps that are used to stabilize the lubricating compositions may be varied. Generally in pre-

paring greases, a fatty oil is mixed with a mineral oil, heated, and an alkali added to saponify the fatty oil and after all of the fatty oil has been saponified a metallic soap separately prepared is added. In manufacturing a compounded oil, however, the metallic soaps are either separately prepared and then added to the mineral oil, or prepared in one operation in which the two different metallic salts may be added to an alkali soap and both metallic soaps formed simultaneously.

A method of preparing a compounded oil is as follows:

10% of lead oleate is dissolved in mineral oil along with 1% of the desired soap. The temperature may be raised slightly to dissolve the soaps in the oil. The composition of the compounded oil is as follows:

|                            | Per cent |
|----------------------------|----------|
| 20 Mineral lubricating oil | 89.0     |
| Lead oleate                | 10.0     |
| Cadmium or cobalt oleate   | 1.0      |

The foregoing description is merely illustrative and various changes and alternative arrangements may be made within the scope of the

appended claims in which it is our intention to claim all novelty inherent in the invention as broadly as the prior art permits.

We claim:

1. A stable lubricating composition comprising a mineral oil, a soap in grease forming proportion selected from the group consisting of alkali, alkaline earth and lead soaps, and less than 2½% of a metallic soap selected from the group consisting of cobalt oleate, cobalt linoleate, cobalt 10 naphthenate, cobalt soaps of fatty acids obtained by oxidizing paraffin wax, cadmium oleate, cadmium linoleate, cadmium naphthenate, cadmium soaps of fatty acids obtained by oxidizing paraffin wax and manganese linoleate. 15

2. A stable lubricating composition according to claim 1 in which the alkaline earth soap is a calcium soap.

3. A stable lubricating composition according to claim 1, in which the alkali metal soap is a 20 sodium soap.

4. A stable lubricating composition according to claim 1, in which the lead soap is lead oleate.

FLOYD L. MILLER.

ARNOLD J. MORWAY. 25